

# United States Patent Office

2,710,841  
Patented June 14, 1955

1

2,710,841

## METHOD OF PREPARING SUBSTITUTED UREA-THICKENED GREASES

Edward A. Swakon, Hammond, and Cecil G. Brannen, Munster, Ind., assignors to Standard Oil Company, Chicago, Ill., a corporation of Indiana

No Drawing. Application November 18, 1953,  
Serial No. 392,996

24 Claims. (Cl. 252—51.5)

The present invention relates to an improved method of manufacturing lubricant greases. More particularly, it relates to a novel process for the manufacture of greases comprising a lubricant vehicle thickened with one or more alkyl or aryl-substituted ureas.

As lubricants are required to perform at higher and higher temperatures because of increased speeds of engines and machines, the advent of jet propulsion, atomic energy as a source of power, etc., it has become increasingly difficult to prepare greases fulfilling the re-

2

employed at temperatures as high as about 450° F., other lubricant vehicles, either natural or synthetic, may also be thickened with these materials to produce greases of particular utility over a wide range of temperatures.

In copending application for Letters Patent S. N. 393,010 filed November 18, 1953 (which is also a continuation in part of S. N. 318,321), greases prepared with thickeners comprising mixtures of at least two different aryl substituted ureas and/or diureas are described and claimed. Thus, in accordance with the invention described in said application, mixtures of aryl substituted ureas prepared by reacting (1) at least two different aryl isocyanates with at least one aryl amine (mono- or diamine) or (2) at least two different aryl monoamines with at least one aryl isocyanate (mono- or diisocyanate). Thus, greases are prepared in accordance with the later filed application which comprises an oleaginous lubricant vehicle thickened with mixtures of aryl substituted ureas prepared, for example, as follows:



quirements of such lubricants. In attempting to provide such greases, the art has progressed from the use of petroleum lubricant vehicles thickened with metal soaps of long chain fatty acids, e. g. lithium hydroxystearate, to more thermally stable synthetic lubricating oils such as the aliphatic diesters of dicarboxylic acids, silicone polymers, etc., thickened with such soaps or inorganic materials such as silica gels. The progress of thickener research has not in general, however, kept pace with the development of lubricant vehicles. And at temperatures as high as 400° to 450° F. there are few if any greases available which will retain their consistency and lubricity for any substantial period of time.

In recent years various synthetic lubricant vehicles, e. g. the silicones, fluorocarbons, etc., have been found to be potentially valuable for use in greases employed at higher temperatures because of their thermal stability and relatively low volatility. Unless, however, a thickener having substantially the same degree of thermal stability is available to produce a grease from such an oil, they are of little use.

In our copending application for Letters Patent S. N. 318,321, filed November 1, 1952 (of which the present application is a continuation in part), it is disclosed that certain very high melting aromatic ureas, diureas, amides, and diamides, all of which contain at least one



radical wherein R is an aryl radical; and which are referred to broadly as aryl carbamyl compounds, may be employed to thicken silicone polymer oils, as well as other known lubricant vehicles to produce greases which are stable and display excellent lubricant properties over a wide range of temperatures. Whereas silicone polymer oils are particularly preferred for use in greases

40 Wherein R and R' are different aryl or substituted aryl radicals. R'' represents an aryl or substituted aryl radical which may be same as or different from R and R'. These may differ in that one may be unsubstituted and the other substituted, or both may be substituted but by different functional groups, e. g. by groups such as nitro-, halo-, alkyl, aryl, alkylaryl, arylalkyl, sulfonyl, carboxyl, hydroxyl, amido, sulfonamido, etc. or one may be monocyclic and the other polycyclic, e. g. phenyl, diphenyl, naphthyl, etc. Instead of the reactants being limited to two amines and one isocyanate or vice versa, 50 as shown, the reactants may comprise a plurality of both amines and isocyanates and there may be both mono- and di-substituted compounds of each class present in a given reaction. Thus, for example, an especially outstanding thickener may be prepared by reacting p-biphenyl isocyanate with p-phenylene diamine and benzidine, e. g. in a molar ratio of 4:1:1 respectively. To such a reaction mixture there may be added one or more additional isocyanate, e. g. p-chlorophenyl isocyanate. Examples of other reactants and the products obtainable 55 therefrom will be hereinafter set forth. R'' is a divalent arylene radical, e. g. phenylene, biphenylene, naphthylene, etc. which may be substituted by such hydrocarbon or functional groups as are above enumerated with respect to R, R', and R''.

60 It has been discovered that improved, high consistency greases of the type claimed in the foregoing copending applications can be prepared with substantial savings in the amount of thickener employed by preparing the substituted urea thickeners by chemical reaction in the lubricating oil vehicle.

Furthermore, related greases embodying alkyl substituted urea thickeners can readily be prepared by this technique. And whereas, for purposes of illustration, the following detailed description will refer particularly

to the preparation of aryl substituted urea thickened greases, it should be understood that the invention is broadly concerned with an improved method of preparation of greases which comprise lubricant vehicles thickened by alkyl substituted ureas and/or ureas substituted by both aryl and alkyl radicals, as well. These latter thickeners will also be described in greater detail.

For purposes of illustration, therefore, an aryl urea thickened grease is prepared in accordance herewith by first introducing the amine component or components dissolved in an organic solvent to a solution of the isocyanate or isocyanates in the lubricant vehicle, e. g. a silicone oil. Various solvents may be used. Their requirements are that they be chemically inert with respect to the vehicles and reactants, that they boil at a temperature permitting ready removal from the grease preferably substantially below 300° F., and that they dissolve substantially completely the reactants employed to produce the ureas. An immediate reaction occurs at room temperature to produce the arylurea thickener during rapid agitation of the mixture. Higher temperatures may be employed if desired. When reaction is complete, the solvent, e. g. dioxane, chloroform, benzene, ethyl acetate, 2-butanone, etc., is removed, preferably by heating at atmospheric pressure (vacuum may be employed if desired.) The solvent-free grease may then be milled to produce a smooth homogeneous product. But it is preferred, and especially with arylurea thickened silicone oils intended for use at very elevated temperatures, that the grease be heated after solvent removal and preferably before milling to the highest proposed operating temperature at which the grease is ultimately to be employed (this will depend particularly on the thermal stability of individual oil and thickener) and it is retained at such temperature for a period of time which may vary from about 30 minutes to about 72 hours. After the heating step is complete, the grease is cooled to room temperature and milled. The resulting greases are smooth and buttery in texture and have excellent thermal stability. Whereas it is preferred that the isocyanate be dissolved in the lubricant vehicle and the amine component be added thereto in a solvent, this procedure may be reversed with the amine being dissolved and/or melted in the oil and the isocyanate being added via the solvent.

It has been found that improved greases may be manufactured, in accordance herewith, by preparing (by chemical reaction) the thickener in situ in the lubricant vehicle in the absence of a solvent. But it is preferred to employ a solvent because the same contributes in large measure to the completeness of the reaction of isocyanate and amine and the dispersion of resulting thickener throughout the oil. In cases where one or more of the reactants is a solid, e. g. 4-biphenyl isocyanate (p-xenyl isocyanate), it may be heated in the oil until melted or it may be dissolved in the solvent first and then added to the oil either before or simultaneously with the amine.

In accordance with the present invention, lubricating vehicles such as silicone polymer oils, mineral lubricating oils derived from petroleum, synthetic lubricating oils such as polyalkylene glycols and their derivatives, dicarboxylic esters, fluorocarbons, etc. and preferably the silicone polymer oils may be thickened to grease consistency by thickeners of the type described herein prepared by chemical reaction in the lubricating oil itself. Amounts of such thickeners of from 5 to 70% and preferably from about 10 to 50% may be employed. Thus, in accordance herewith, substituted urea thickeners comprising one or more of the following type compounds (designated by general formula) are prepared in lubricating oils in an amount sufficient to thicken such oil to grease consistency.



In the above formulae, R and R' represent aryl or alkyl radicals which may be the same or different. These radicals may be substituted or unsubstituted, e. g. by substituent groups such as nitro-, halo-, alkyl-, aryl-, alkylaryl-, arylalkyl-, sulfonyl-, carboxyl-, hydroxyl-, amido-, sulfonamido, etc.; where aryl they may be mono- or polycyclic, e. g. phenyl, diphenyl, naphthyl, etc. R'' is a divalent aryl or alkyl radical (i. e. an arylene or alkylene radical) such as phenylene, biphenylene, naphthylene, ethylene, propylene, nonylene, etc., which may be substituted by such hydrocarbon or other substituent groups as are above enumerated with respect to R and R'. Where alkyl or substituted alkyl radicals are employed, the number of carbon atoms therein may vary from 1 to about 30 and preferably from 2 to about 10 carbon atoms. R'', when alkyl, may have from 2 to about 20 carbon atoms and preferably from 2 to about 10.

Obviously, a wide variety of such ureas may be produced in accordance herewith and these are dependent upon the number and type of isocyanate and amine reactants selected. Thus, by way of illustration and not of limitation, a number of isocyanates which may be employed in accordance with the present invention to produce such greases are set forth below. And it should be understood, as indicated above, that the reactants may be selected so as to produce either mixtures of alkyl and/or aryl-substituted ureas or individual alkyl or aryl-substituted ureas and they may be mono- or poly-ureas.

Suitable aryl isocyanates which may be employed in accordance herewith are p-chlorophenyl isocyanate, p-tolyl isocyanate, tolylene diisocyanate, p-biphenyl isocyanate (p-xenyl isocyanate), phenyl isocyanate, p-carboxyphenyl isocyanate,  $\alpha$ -naphthyl isocyanate, p,p'-diisocyanato-biphenyl, 1,4-diisocyanato-benzene, 2,5-dichlorophenyl isocyanate, o-biphenyl isocyanate (o-xenyl isocyanate), o-chlorophenyl isocyanate, p,p'-diisocyanatodi-phenylmethane, etc.

Examples of alkyl isocyanates which may be employed are hexyl isocyanate, chlorononyl isocyanate, 1,6-di-isocyanato hexane, 1,12-di-isocyanato dodecane, cyclohexyl isocyanate, octadecyl isocyanate, etc.

Examples of suitable aryl amines are p-aminobenzoic acid, p-aminobiphenyl, benzidine, dianisidine, o-tolidine, p-aminophenol, p-aminobenzonitrile, p-phenylene diamine, m-phenylene diamine, o-phenylene diamine, 2,5-dichloroaniline, aniline, p-toluidine, etc.

Typical of the alkyl amines which may be employed are hexylamine, dodecylamine, octylamine, nonylamine, cyclohexylamine, chlorodecylamine, 1,6-di-amino hexane, 1,10-diamino-decane, 1,3-diamino propane, diethylene triamine, triethylene tetramine, etc.

The above enumerated amines and isocyanates, as well as others not specifically referred to but which will be readily suggested to one skilled in the art as result of the examples given, may be reacted to produce a wide variety of mono- and/or diureas. Thus, if symmetrical monoureas or diureas are desired, either an amine and an isocyanate having the same hydrocarbon radical may be reacted or, for example, a single isocyanate may be reacted with a diamine. On the other hand, for example, if mixtures of aryl substituted ureas of the type claimed in S. N. 393,010 filed November 18, 1953 are desired, then at least one amine and at least two isocyanates or vice versa must be reacted. From such as this latter mixture of reactants, a thickener comprising a mixture of different ureas would necessarily result.

The silicone polymer oils which may be employed in accordance with the present invention are those falling substantially within the lubricating oil viscosity range.

In general, such oils have the following unit structure:



75 wherein R and R' represent substituted or unsubstituted

alkyl, aryl, alkylaryl, arylalkyl, or cycloalkyl radicals. Such compounds may be produced by well-known method, e. g. the hydrolysis of dialkyldichlorosilanes or dialkyldiethoxysilanes with a suitable chain stopper, e. g. a tri-substituted mono-chlorosilane. For purposes of the present invention, those polymers which are high boiling liquids within the lubricating oil viscosity range are suitable, these generally possessing a viscosity at 100° F. which is within the range of from about 25 to about 3500 S. S. U. It is preferred, for purposes hereof, to employ such oils as have a viscosity at 100° F. of from about 100 S. S. U. to about 1250 S. S. U. Such products are generally colorless and inert, have a very low volatility and undergo relatively slight change in viscosity for a given change in temperature. Relatively common oils of this type are dimethylsilicone polymer, phenylmethylsilicone polymer, chlorophenylmethylsilicone polymer, etc., it being preferred to employ the phenylmethylsilicone polymer in accordance herewith. Methods of preparing such compounds are taught in numerous patents, e. g. U. S. 2,410,346, U. S. 2,456,496, and in the literature such as "Chemistry of the Silicones" by Rochow, page 61, et seq. A particularly desirable phenylmethylsilicone polymer for use in accordance with the present invention is Dow-Corning 550 Silicone Fluid, a product of Dow-Corning, Inc., which has a viscosity at 100° F. of about 300 to about 400 S. S. U. Another is Dow Corning 510 Silicone Fluid, etc.

Other oleaginous lubricant vehicles which may be employed herewith are, for example, mineral oils in the lubricating oil viscosity range, i. e. from about 50 S. S. U. at 100° F. to about 300 S. S. U. at 210° F. These mineral oils are preferably solvent extracted, to substantially remove the low V. I. constituents, e. g. aromatics, with phenol, furfural, B,B'-dichlorodiethylether(Chlorex), liquid SO<sub>2</sub>, nitrobenzene, etc. Synthetic lubricating oils resulting from polymerization of unsaturated hydrocarbons or other oleaginous materials within the lubricating oil viscosity range such as high molecular weight polyoxyalkylene compounds such as polyalkylene glycols and esters thereof, aliphatic diesters of dicarboxylic acids such as the butyl, hexyl, 2-ethylhexyl, decyl, lauryl, etc. esters of sebacic acid, adipic acid, azelieic acid, etc., may be thickened by the ureido compounds of the present invention to produce excellent greases. Polyfluoro derivatives of organic compounds, particularly hydrocarbons, in the lubricating oil viscosity range have shown excellent promise when thickened with compounds of the present invention. Thus, any lubricating oil, natural or synthetic, which when thickened in accordance herewith, will result in a useful lubricant grease, may be employed in accordance herewith. Mixtures of these various vehicles may be employed if desired. Thus, for example, a mixture of diester and fluorocarbon; of various silicone fluids; a diester and a hydrocarbon oil; etc. may be employed.

The following are detailed working examples illustrative of the present novel method of grease manufacture as applied to the preparation of aryl ureas. The characteristics and thermal stability of the greases so prepared, as well as others prepared in like manner, are compared in Table 1 with greases of the same general type, i. e. arylurea thickened greases prepared by milling a prepared arylurea thickener with an oil. The greater consistency obtained with substantially less thickener by the use of the present novel method is striking.

#### EXAMPLE 1

A five-gallon double-action scraper kettle was charged with 2000 grams of D. C. 550 Silicone Fluid (phenylmethylpolysiloxane product of Dow Corning more fully defined hereinabove), 160 grams of p-chlorophenyl isocyanate, and 204 grams of p-biphenyl isocyanate. The mixture was heated to 150° F. to melt the p-biphenyl isocyanate.

To the above stirred mixture, 184 grams of benzidine

dissolved in about 2 liters of 2-butanone was added over a period of 20 minutes.

The remainder of the silicone oil, 1000 grams, was then added and the solvent was boiled off and the resulting grease was heated with stirring for 4 hours at 420° F. After the grease was cooled to room temperature, it was passed through a colloid mill to complete the preparation. The finished grease had an ASTM penetration of 318 (unworked) (Kaufmann micropenetration of 132), 338 after 60 strokes, and 354 after 100,000 strokes. An A. B. E. C.-N. L. G. I. bearing test (hereinafter described) employing this grease at 450° F. and 10,000 R. P. M. ran for 553 hours.

#### EXAMPLE 2

A mixture of 13.1 grams of p-biphenyl isocyanate dissolved in 92 grams of solvent extracted SAE-20 petroleum lubricating oil was introduced to a beaker; 9.9 grams of 1,2-propylene diamine was added thereto with stirring. The resulting soft, grainy paste was heated overnight at a temperature of 250° F. and then milled to produce a grease having a micropenetration of 131. The heating and milling steps were repeated and the micro-penetration at the conclusion thereof had gone up to 162.

#### EXAMPLE 3

A solution of 9.8 grams of p-biphenyl isocyanate in 50 milliliters of ethyl acetate was added with stirring to a mixture in a beaker comprising 12.8 grams of cetylamine, 60.8 grams of solvent extracted SAE-20 petroleum lubricating oil and a substantial amount of ethyl acetate. The resulting mixture was milled in a roller mill to produce a rather soft buttery grease.

#### EXAMPLE 4

A hot solution consisting of 276 grams of benzidine, 162 grams of p-phenylene diamine and two liters of ethyl acetate was poured rapidly into a solution of 10.8 pounds of D. C. 550 Silicone Fluid and 788 grams of p-tolyl isocyanate in the kettle referred to in Example 1. The mixture immediately thickened. After the solvent was removed by distillation, the mix was heated to about 420° F. and kept at this temperature for about four hours. The grease was then allowed to cool overnight without stirring and finally finished by milling. The resulting grease was smooth, opaque paste having an ASTM penetration of 300 (Kaufmann micropenetration -81).

#### EXAMPLE 5

The five-gallon, double-action scraper kettle was charged with 9.46 pounds of D. C. 550 Silicone Fluid and 780 grams of p-biphenyl isocyanate. This mixture was heated to 160° F. in order to melt the isocyanate and make a homogeneous solution. A solution consisting of 184 grams of benzidine, 108 grams of p-phenylene diamine and 1500 grams of ethyl acetate was then poured very rapidly into the kettle. The mixture thickened immediately. The cover was then bolted in place and the kettle was heated by introducing 100 p. s. i. steam to the kettle jacket to raise the mixture to a temperature of about 320° F. The solvent was recovered by condensing it in a copper coil which was submerged in water bath. After the solvent was removed, the kettle was uncovered and heated electrically to 425° F. and kept at this temperature for one hour. The grease was allowed to cool overnight without stirring, and then milled. The resulting grease was a purple, smooth, opaque paste. Thickener concentration was 20%. ASTM Penetration: Unworked -318; worked -320.

The bearing test referred to in Example 1 above is a tentative one adopted by the Coordinating Research Council during the last war and is generally referred to as the A. B. E. C.-N. L. G. I. Test. It is conducted as follows:

3 grams of grease are placed in each of two bearings disposed on the test spindle. One bearing, a special heat

treated precision 204 K Norma-Hoffman (or Marlin-Rockwell) bearing, is subjected to a temperature of 450° F. in an oven, the other bearing, a standard New Departure 204 K bearing, is at a sufficiently low temperature to avoid any failure due to thermal stability of the grease. Temperature is determined by a thermocouple inserted in the grease between the races of the bearing in the oven. Failure is adjudged to occur when (1) the temperature in the test bearing reaches 470° F. or higher, (2) wattage in excess of 300% of normal wattage is required, or (3) the bearing does not turn over at the beginning of a test cycle (the test is conducted in cycles of 20 hours operating and 4 hours at rest).

In Table 1 the term "In situ" is employed to designate grease preparation by the method of the present invention as exemplified by illustrative examples 1, 2, and 3 above. The compound in parentheses following this term is the solvent employed. The term "solid milled" refers to grease preparation wherein the thickener is first prepared and then mixed and milled with the oil. The lubricant vehicle employed in the greases shown in Table 1 was D. C. 550 Silicone Fluid.

Table 1

| Thickener |         | Method of Preparation | Micropenetration (Kaufmann) |
|-----------|---------|-----------------------|-----------------------------|
| Kind      | Percent |                       |                             |
| A         | 30      | Solid milled          | 450+                        |
| A         | 10      | In situ (benzene)     | 110                         |
| A         | 15      | In situ (2-butanone)  | 47                          |
| B         | 30      | Solid milled          | 212                         |
| B         | 20      | In situ (chloroform)  | 77                          |
| C         | 30      | Solid milled          | 450+                        |
| C         | 15      | In situ (2-butanone)  | 75                          |
| C         | 15      | In situ (dioxane)     | 82                          |

A—product of the reaction of 1 equivalent of p-chlorophenyl isocyanate, 1 equivalent of p-biphenyl isocyanate, and 1 equivalent of benzidine.

B—product of the reaction of 2 equivalents of p-biphenyl isocyanate and 1 equivalent of benzidine.

C—product of the reaction of 2 equivalents p-chlorophenyl isocyanate and 1 equivalent of benzidine.

While the reasons are not fully understood, the particular solvent employed as well as the amount thereof and the time the grease is in contact therewith appear to have a definite effect on the quality of greases prepared in accordance herewith. Experiments were run to determine the effect of concentration of reactants and effect of prolonged contact of solvent with the grease. Particle size measurements were used to evaluate the techniques. It was found that the smaller the particle size, the higher the consistency of the grease, i. e. consistency is roughly determined by particle size when comparing greases of the same composition and thickener percentage. The data in Table 2 demonstrate this for certain greases prepared by the technique of the present invention employing D. C. 550 Silicone Fluid lubricant vehicle.

Table 2

| 5 | Thickener |         | Micropenetration (Kaufmann) | Average Particle Length ( $\mu$ ) |
|---|-----------|---------|-----------------------------|-----------------------------------|
|   |           | Percent |                             |                                   |
| A |           | 20      | 55                          | 0.16                              |
| A |           | 20      | 113                         | 0.57                              |
| B |           | 15      | 139                         | 0.44                              |
| B |           | 15      | 249                         | 0.60                              |
| C |           | 15      | 132                         | 0.66                              |
| C |           | 15      | 203                         | 0.75                              |

A—2 moles p-tolyl isocyanate + 1 mole benzidine prepared with dioxane solvent.

B—2 moles p-chlorophenyl isocyanate + 1 mole benzidine prepared with 2-butanone solvent.

C—1 mole p-chlorophenyl isocyanate + 1 mole p-biphenyl isocyanate + 1 mole benzidine prepared with 2-butanone solvent.

To further illustrate this point, p-chlorophenyl isocyanate, p-biphenyl isocyanate, and benzidine were reacted in the presence of D. C. 550 in (1) the least amount of 2-butanone and (2) ten times the least amount of solvent which it previously had been determined would dissolve the reactants. Samples were withdrawn at intervals, viz. (1) immediately after mixing, (2) after 10 minutes, and (3) after refluxing for 24 hours. The particle sizes were strikingly different. In all cases, the particles were much larger after the greases had been refluxed for 24 hours and slightly larger 10 minutes after mixing. Furthermore, the particles as initially formed were smaller in the reaction using the least amount of solvent. These experiments were repeated using benzene as the solvent. The same increase in size was observed. In this case, the particles as initially formed were smaller than those formed initially in 2-butanone.

Accordingly, it is preferred to employ substantially no more solvent than the minimum amount required to dissolve the reactants employed in the production of substituted ureas in accordance herewith. And it is important that the solvent be removed from the thickener-oil mixture as soon as reaction is complete. The time of reaction cannot be known for all cases, but since the ureido compounds are usually formed substantially at once under adequate mixing conditions and the use of sufficient solvent, the solvent should be removed within about one-half hour and preferably within about 15 minutes from the time all the reactants had been admixed in the reaction medium.

As indicated above, the present method for preparing substituted urea greases is applicable to a variety of lubricant vehicles. In Table 3 are listed greases prepared by the present technique in vehicles other than silicone polymer oils. An ethyl acetate solvent was employed in each preparation.

Certain greases of the type set forth in Table 3 are stable at relatively high temperatures, e. g. 300 to 350°

Table 3

| Thickener                                                                   | Percent | Oil                                                 | Viscosity at 100° F. Cstks. | Grease, Micropenetration |
|-----------------------------------------------------------------------------|---------|-----------------------------------------------------|-----------------------------|--------------------------|
| 1. {1,4-Bis-(3-phenylureido)-benzene<br>1,4'-Bis-(3-phenylureido)-biphenyl} | 20      | Di-2-ethylhexyl sebacate <sup>1</sup>               | 22.2                        | 80                       |
| 2. {1,4-Bis-(3-phenylureido)-benzene<br>1,4'-Bis-(3-phenylureido)-biphenyl} | 20      | Solvent extracted SAE 20 petroleum lubricating oil. | 70.7                        | 117                      |
| 3. {1,4-Bis-(3-phenylureido)-benzene<br>1,4'-Bis-(3-phenylureido)-biphenyl} | 15      | Solvent extracted SAE 40 petroleum lubricating oil. | 174.9                       | 243                      |
| 4. {1,4-Bis-(3-phenylureido)-benzene<br>1,4'-Bis-(3-phenylureido)-biphenyl} | 15      | Orthosilicate ester <sup>2</sup>                    | 6.9                         | 203                      |
| 5. {1,4-Bis-(3-phenylureido)-benzene<br>1,4'-Bis-(3-phenylureido)-biphenyl} | 10      | Fluorocarbon <sup>3</sup>                           | 195.6                       | 64                       |
| 6. {1,4-Bis-(3-phenylureido)-benzene<br>1,4'-Bis-(3-phenylureido)-biphenyl} | 20      | Di-2-ethylhexyl sebacate                            | 12.7                        | 148                      |
| 7. 1,2-Bis-[3-(4-biphenyl)-ureido]-propane                                  | 20      | Solvent extracted SAE 20 petroleum lubricating oil. | 70.7                        | 162                      |
| 8. 4,4'-Bis-(3-phenylureido)-biphenyl                                       | 12      | Fluorocarbon <sup>4</sup>                           | 2,000                       | 95                       |

<sup>1</sup> In addition to the di-(2-ethylhexyl) sebacate, which comprises 90.6% of the vehicle, there is present Acryloid HF-825, 3.9%; phenothiazine, 0.5%; trioresyl phosphate, 5.0%; silicone anti-foam, 0.001%.

<sup>2</sup> Orsil BF-1-S<sup>3</sup> (product of Oronite Chemical Corp.).

<sup>3</sup> A mixture comprising 41% "Fluorolube" (OP-320-52) D-8433 (an experimental product of Hooker Chemical Co.) and 59% of "Kel-F-40" (product of The M. W. Kellogg Co.).

<sup>4</sup> "Kel-F-40"—Product of The M. W. Kellogg Co.

F. and higher, but are generally useful at temperatures somewhat below those at which greases embodying a silicone oil as the lubricant vehicle, may be employed. Greases of the type herein described, particularly embodying a petroleum lubricating oil, are useful at temperatures encountered in normal automotive or industrial uses and admirably fulfill the requirements of a multipurpose grease.

Whereas the substituted urea thickeners employed in accordance herewith have been prepared in each instance by the reaction of an amine with an isocyanate, such materials may be prepared by other reactions and it should be understood that this invention is not limited to the preferred described chemical reaction (i. e. amine-isocyanate) for producing such thickeners. Thus, for example, ureido compounds of the type herein described may be prepared by the reaction of an amine with an acid azide or a substituted carbamyl chloride rather than an isocyanate as herein described. From the reaction of an acid azide with an amine, nitrogen is evolved whereas from the reaction of a carbamyl chloride with an amine, hydrogen chloride is a by-product. The evolution of hydrogen chloride has certain disadvantages in the present in situ method of producing greases. And accordingly, its use, generally, is not recommended. The azide-amine reaction, however, will produce a suitable grease thickener with nitrogen evolution and since nitrogen is inert, such a reaction may readily be employed in accordance herewith.

Percentages given herein and in the appended claims are by weight unless otherwise specified.

The greases of the present invention may contain added constituents such as antioxidants, oiliness agents, extreme pressure additives, etc. without in any way departing from the scope of the present invention.

Having thus described our invention, what we claim as novel and desire to protect by Letters Patent is as follows:

1. The method of manufacturing a lubricant grease comprising a substituted urea-thickened lubricant vehicle which comprises producing in situ in a reaction medium comprising the lubricant vehicle of the grease substituted urea selected from the group consisting of



and mixtures thereof wherein R and R' represent hydrocarbon radicals selected from the class consisting of aryl, alkyl, and substituted aryl, said aryl radicals having no more than 12 cyclic carbon atoms and said alkyl radicals having from 1 to 30 carbon atoms, and R'' represents a hydrocarbon radical selected from the class consisting of alkylene, arylene, substituted alkylene, and substituted arylene radicals, said alkylene radicals having from 2 to about 20 carbon atoms and said arylene radicals having no more than 12 cyclic carbon atoms, said substituted urea being prepared in an amount sufficient to thicken the amount of lubricant vehicle in which it is prepared.

2. The method of claim 1 wherein the ultimate mixture of substituted urea and lubricant vehicle is milled.

3. The method of claim 1 wherein said substituted urea is formed in situ in said lubricant vehicle by chemical reaction in said lubricant vehicle of a mixture comprising a compound selected from the group consisting of RNCO, OCNR'NCO and mixtures thereof and a compound selected from the group consisting of R''NH<sub>2</sub> and H<sub>2</sub>NR'''NH<sub>2</sub> in which R and R'' are hydrocarbon radicals selected from the group consisting of alkyl radicals having from 1 to about 30 carbon atoms and aryl and substituted aryl radicals having no more than 12 cyclic carbon atoms, and R' and R''' are hydrocarbon radicals selected from the group consisting of alkylene and substituted alkylene radicals having from 2 to about 20 carbon

atoms and arylene and substituted arylene radicals having no more than 12 cyclic carbon atoms.

4. The method of claim 3 wherein the reactants from which the aryl-substituted urea is produced comprise p-chlorophenyl isocyanate, p-biphenyl isocyanate and benzidine.

5. The method of claim 3 wherein the reactants from which the aryl-substituted urea is produced comprise p-tolyl isocyanate, p-phenylene diamine and benzidine.

6. The method of claim 3 wherein the reactants from which the aryl-substituted urea is produced comprise p-biphenyl isocyanate, p-chlorophenyl isocyanate, p-phenylene diamine, and benzidine.

7. The method of manufacturing a lubricant grease comprising a substituted urea-thickened lubricant vehicle which comprises producing in situ in a reaction medium comprising the lubricant vehicle of the grease substituted urea selected from the group consisting of



and mixtures thereof wherein R and R' represent hydrocarbon radicals selected from the class consisting of aryl, alkyl, and substituted aryl, said aryl radicals having no more than 12 cyclic carbon atoms and said alkyl radicals having from 1 to 30 carbon atoms, and R'' represents a hydrocarbon radical selected from the class consisting of alkylene, arylene, substituted alkylene, and substituted arylene radicals, said alkylene radicals having from 2 to about 20 carbon atoms and said arylene radicals having no more than 12 cyclic carbon atoms, said substituted urea being prepared in an amount sufficient to thicken the amount of lubricant vehicle in which it is prepared, and heating the mixture of substituted urea and lubricant vehicle to a temperature within the range of from about 150° F. to about 450° F. for a period of about 1/2 hour to a period of 72 hours.

8. The method of claim 7 wherein the ultimate mixture of substituted urea and lubricant vehicle is milled.

9. The method of manufacturing a lubricant grease comprising a substituted urea-thickened lubricant vehicle which comprises producing in situ in a reaction medium comprising the lubricant vehicle of said lubricant grease and an organic solvent having a boiling point below about 300° F. in which solvent the reactants from which the substituted urea is produced are substantially completely soluble, substituted urea selected from the group consisting of



and mixtures thereof where R and R' represent hydrocarbon radicals selected from the class consisting of aryl, alkyl, and substituted aryl, said aryl radicals having no more than 12 cyclic carbon atoms and said alkyl radicals having from 1 to 30 carbon atoms, and R'' represents a hydrocarbon radical selected from the class consisting of alkylene, arylene, substituted alkylene, and substituted arylene radicals, said alkylene radicals having from 2 to about 20 carbon atoms and said arylene radicals having no more than 12 cyclic carbon atoms, said substituted urea being prepared in an amount sufficient to thicken to grease consistency the amount of lubricant vehicle in which it is prepared, and then removing said solvent.

10. The method of claim 9 wherein the ultimate mixture of substituted urea and lubricant vehicle is milled.

11. The method of manufacturing a lubricant grease comprising a substituted urea-thickened lubricant vehicle which comprises producing in situ in a reaction medium comprising the lubricant vehicle of said lubricant grease

## 11

and an organic solvent having a boiling point below about 300° F. in which solvent the reactants from which the substituted urea is produced are substantially completely soluble, substituted urea selected from the group consisting of



and mixtures thereof wherein R and R' represent hydrocarbon radicals selected from the class consisting of aryl, alkyl, and substituted aryl, said aryl radicals having no more than 12 cyclic carbon atoms and said alkyl radicals having from 1 to 30 carbon atoms, and R'' represents a hydrocarbon radical selected from the class consisting of alkylene, arylene, substituted alkylene, and substituted arylene radicals, said alkylene radicals having from 2 to 20 carbon atoms and said arylene radicals having no more than 12 cyclic carbon atoms, said substituted urea being prepared in an amount sufficient to thicken to grease consistency the amount of lubricant vehicle in which it is prepared, removing said solvent, and heating the remaining mixture of substituted urea and lubricant vehicle to a temperature within the range of from about 150° F. to about 450° F. for a period of from about 1/2 hour to a period of 72 hours.

12. The method of claim 11 wherein the ultimate mixture of substituted urea and lubricant vehicle is milled.

13. The method of claim 11 wherein the organic solvent comprises dioxane.

14. The method of claim 11 wherein the solvent comprises 2-butanone.

15. The method of claim 11 wherein the solvent comprises benzene.

16. The method of manufacturing a lubricant grease comprising an aryl substituted urea-thickened lubricant vehicle, which method comprises forming in situ, in a reaction medium comprising the lubricant vehicle of said lubricant grease, aryl substituted urea having the general formula



in which R and R' are aryl radicals containing no more than 12 cyclic carbon atoms selected from the group consisting of aryl and substituted aryl radicals, said aryl substituted urea being prepared in an amount sufficient to thicken to grease consistency the amount of lubricant vehicle in which it is prepared.

17. The method of manufacturing a lubricant grease comprising an aryl substituted urea-thickened lubricant vehicle, which method comprises forming in situ, in a reaction medium comprising the lubricant vehicle of said lubricant grease, aryl substituted urea having the general formula



in which R and R' are aryl radicals containing no more than 12 cyclic carbon atoms selected from the group consisting of aryl and substituted aryl radicals, said aryl substituted urea being prepared in an amount sufficient to thicken to grease consistency the amount of lubricant vehicle in which it is prepared, adding additional lubricant vehicle to said urea-thickened lubricant vehicle and heating said resultant mixture to a temperature in the range of from 150° F. to about 450° F. for a period of from 1/2 hour to about 72 hours.

18. The method of claim 17 wherein the ultimate mixture of substituted urea and lubricant vehicle is milled.

19. The method of manufacturing a lubricant grease comprising an aryl substituted urea-thickened lubricant vehicle, which method comprises forming in situ, in a reaction medium comprising the lubricant vehicle of said

5 lubricant grease, aryl substituted urea having the general formula



in which R and R' are aryl radicals containing no more than 12 cyclic carbon atoms selected from the group consisting of aryl and substituted aryl radicals, and R'' is a divalent radical containing no more than 12 cyclic carbon atoms selected from the group consisting of arylene and substituted arylene radicals, said aryl substituted urea being prepared in an amount sufficient to thicken to grease consistency the amount of lubricant vehicle in which it is prepared.

10 20. The method of manufacturing a lubricant grease comprising an aryl substituted urea-thickened lubricant vehicle, which method comprises forming in situ in a reaction medium comprising the lubricant vehicle of said lubricant grease a mixture of aryl substituted urea having the general formula



and aryl substituted urea having the general formula



25 in which R and R' are aryl radicals containing no more than 12 cyclic carbon atoms selected from the group consisting of aryl and substituted aryl radicals and R'' is a divalent radical containing no more than 12 cyclic carbon atoms selected from the group consisting of arylene and substituted arylene radicals, said mixture of substituted ureas being prepared in an amount sufficient to thicken to grease consistency the amount of lubricant vehicle in which it is prepared.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 94

## 13

is a divalent radical containing no more than 12 cyclic carbon atoms selected from the group consisting of arylene and substituted arylene radicals, said substituted urea being prepared in an amount sufficient to thicken to grease consistency the amount of lubricant vehicle in which it is prepared, heating the mixture of arylurea, lubricant vehicle, and organic solvent to substantially completely remove said solvent, further heating the solvent-free mixture of arylurea and lubricant vehicle to a temperature within the range of from 150° F. to about 450° F. for a period of from 1/2 hour to about 72 hours, cooling said mixture, and milling said cooled mixture.

23. The method of manufacturing a lubricant grease comprising an alkyl substituted urea-thickened lubricant vehicle, which method comprises forming in situ, in a 15 reaction medium comprising the lubricant vehicle of said lubricant grease, alkyl substituted urea having the general formula



in which R and R' are alkyl radicals having from 1 to about 30 carbon atoms, said alkyl substituted urea being

10

## 14

prepared in an amount sufficient to thicken to grease consistency the lubricant vehicle in which it is prepared.

24. The method of manufacturing a lubricant grease comprising an alkyl substituted urea-thickened lubricant vehicle, which method comprises forming in situ, in a reaction medium comprising the lubricant vehicle which of said lubricant grease, alkyl substituted urea having the general formula



in which R and R' are alkyl radicals having from 1 to about 30 carbon atoms and R'' is selected from the group consisting of alkylene and substituted alkylene radicals having from 2 to about 20 carbon atoms, said alkyl substituted urea being prepared in an amount sufficient to thicken to grease consistency the lubricant vehicle in which it is prepared.

20

## References Cited in the file of this patent

## UNITED STATES PATENTS

2,698,300 Hotten ----- Dec. 28, 1954